

## UNITED STATES PATENT OFFICE

2,454,312

HIGH-STRENGTH CORROSION-RESISTANT  
ALUMINUM ALLOY SHEETS

Thomas L. Fritzlen, Florence, Ala., assignor to  
Reynolds Metals Co., Richmond, Va., a corpora-  
tion of Delaware

No Drawing. Application October 26, 1943,  
Serial No. 507,752

2 Claims. (Cl. 29—197.5)

1

The object of the present invention is to provide a high-strength corrosion-resistant aluminum alloy sheet particularly adapted for aircraft.

It is recognized that sheets rolled from Duralumin types of aluminum alloys, generally containing silicon, copper, manganese and zinc as important constituents, possess high tensile and yield strengths together with suitable elongation factors. Of the alloys of such class, that in very general use, is commercially known as 24S (Cu 4.5%, Mn 0.6%, Mg 1.5%, balance aluminum and normal impurities). By reason of its relatively low resistance to corrosion the said alloy is, for certain aircraft use, clad with pure aluminum. It has, when fully heat treated, a specified tensile strength of 59,000 lbs. per square inch, with a yield strength of 39,000 lbs. per square inch. The product, however, has a marked difference in electrical potential between the core and cladding. In light gauges it requires critical control in solution heat treatment and quenching, and, in a number of other respects, presents difficulties in treatment.

By means of the present invention, an aluminum alloy composition sheet is provided which not only possesses high corrosion resistance, but has greater tensile and yield strengths than the said pure aluminum clad alloy, and less difficulty in treatment. The potential differences between core and cladding are relatively low in the sheet when solution and precipitation heat treated. My product is much less critical with respect to overheating in solution heat treatment.

The characteristic of my aluminum alloy composite sheet is that it consists of a Duralumin type core and a cladding equal to 5%—25% of the composite thickness, the cladding consisting of an aluminum alloy itself of high tensile strength and wholly compatible with the core, in that the core and cladding have substantially equal response to solution heat treatment at given high temperatures, time, quenching conditions and aging conditions.

In making my product, a Duralumin core is prepared, the following general composition being preferred:

TABLE I

|                     | Per cent |
|---------------------|----------|
| Si                  | .75—1.25 |
| Cu                  | 4.0—5.0  |
| Mg                  | .25—.55  |
| Mn                  | .7—1.0   |
| Al and "impurities" | balance  |

NOTE.—When certain other metals are brought into the composition, as by scrap "impurities," it is preferred that the proportions be controlled to the following: Fe .75% max., Cr 25% max., Zn 20% max., and that other "impurities" be controlled to .05% max.

2

The cladding alloy is as follows:

|                   | TABLE II | Per cent |
|-------------------|----------|----------|
| Si                |          | .50—.90  |
| Mg                |          | .8—1.2   |
| Mn                |          | .25—.75  |
| Al and impurities |          | balance  |

NOTE.—When certain other metals are brought into the composition, as by scrap "impurities," it is preferred that the proportions be controlled to the following: Fe .6% max., Cu .05% max., Cr .25% max., and that other "impurities" be controlled to .05% max.

As an example, liner-slabs of the cladding alloy, each amounting to 5% of a core slab, are placed on opposite faces of the latter, and the composite structure rolled into sheet of .064". This sheet 15 may then be subjected to a solution heat treatment which may be at 930—950° F. for about 15—20 minutes, followed by quenching.

For my clad sheet of various gauges, I prefer solution heat treatment for time periods according to the following table:

|               | Gauge | Time    |
|---------------|-------|---------|
| 25            |       | Minutes |
| .020 and .025 |       | 10      |
| .032 and .040 |       | 12      |
| .051 and .064 |       | 15      |
| .072 and .081 |       | 20      |
| .091 and .102 |       | 25      |
| .125 and .156 |       | 30      |
| .188 and .204 |       | 40      |
| .250 and .275 |       | 50      |
| Over .375     |       | 60      |

Specifically, the cladding and other operations may consist of the following:

A core ingot may be cast, say 10" x 40" x 72", the ingot being analyzed, homogenized, hot rolled to 7", and scalped to 6½". The cladding ingot may be cast, say 10" x 40" x 72", analyzed, homogenized, scalped to 9½", hot rolled to .650", cold rolled to .425" and sheared to the size of the scalped core ingot. The core and cladding may then be strapped together, reheated to about 800° F., hot rolled to .265" at said reheating temperature, side trimmed and coiled, cold rolled as in a one stand, four high mill, such as the subject of Steckel's Patent No. 1,779,195, annealed at about 750° F. for two hours, followed by cooling to 500° C. at a rate of 50° per hour, then air quenched, cold rolled in a three stand tandem mill, and cut in sheets, ready for solution heat treatment.

After solution heat treatment, my product may be quenched as in cold water, rolled level and flattened, stretched, side sheared and subjected to a precipitation heat treatment of about 10 hours at 320° F.

Both the core and the cladding obtain high strength through the said solution heat treatment and precipitation heat treatment at elevated temperatures. They are both affected by quenching conditions in the same manner.

My aluminum alloy composite sheet derives its excellent resistance to corrosion for two reasons, namely:

(1) A slower diffusion rate, during solution heat treatment, through the alloy cladding than through a pure aluminum cladding, as determined by heat treating tests and microscopic examination.

(2) Less difference in electric potential between the core and cladding as compared to the same alloy core and a pure metal cladding, as determined through comparative potential measurement, and accelerated corrosion tests in standard  $\text{NaCl}-\text{H}_2\text{O}_2$  solution.

In addition, the following advantages are present in my aluminum alloy composite structure over the currently used aluminum clad 24S alloy:

(a) Easier to hot-roll composite slab and plate.

(b) Easier to cold-roll composite slab and plate.

(c) Lower mechanical properties in annealed condition with subsequent better formability.

(d) Solution heat treatment less critical with respect to solution of soluble constituents and overheating.

(e) Solution heat treatment less critical with respect to quenching.

(f) Quenching of formed aircraft parts after solution heat treatment can be carried out in oil at room temperature or in hot water, avoiding distortion.

(g) Stretching, rolling, and forming can be performed easier in the solution heat treated and quenched condition.

(h) Better welding characteristics.

(i) Lower cost due to use of low Mg content.

(j) Higher endurance limit or fatigue strength.

(k) Less spread in tensile mechanical properties in the fully heat treated condition.

Formed aircraft parts may be made from the sheet, prior to heat solution and precipitation treatment, and these parts given solution heat treatment, say at 935° F., followed by controlled, relatively slow, quenching, as a guard against distortion and subsequent aging, say for 18 hours at 320°, or for 8 hours or for 6-10 hours at 340-350° F.

Cladding may range from 5% to 25% of the composite thickness of the sheet, and the solution heat treatment, quenching and aging may vary in details from the examples given.

In discussion of my clad sheets hereinafter they will be designated "R 301." In the solution heat treatment thereof the tensile properties increase with increasing temperature up to 960 F. and decrease at temperatures over 970° F.

The symbol W hereinafter used defines the heat treated, but not artificially aged, condition of the sheet, and the symbol T defines the heat treated and artificially aged condition of the sheet. The symbol O signifies annealed and soft condition.

Stretching R-301-W sheet 3½ and 5½ per cent raises the tensile and yield strengths appreciably and lowers the elongation when stretching and testing with grain.

Stretching R-301-W 3½ and 5½ per cent with grain raises the "with grain" yield strength and lowers the elongation when aged at 320° F. as compared to R-301-T not prestretched. How-

ever, aging at 350° and 375° F. following pre-stretching R-301-W 3½ and 5½ per cent with grain does not produce consistently higher yield strength.

5 Maximum tensile properties can be obtained upon precipitation heat treatment at any time after solution treatment and quenching. Also, no consistent effect upon corrosion resistance has been noticed when precipitation heat treating at various periods after solution heat treatment.

The precipitation heat treating procedures recommended depend upon several factors; namely, whether further working, dimpling, or forming is to be performed after this treatment and the temperature uniformity of the furnace employed. If further forming is to be performed after precipitation heat treatment, a practice of aging 18 hours at 320° F. is desirable; however, if no further forming is to be carried out, aging for five hours at 360° F. is recommended, if the furnace employed is uniform to plus or minus 5° F. If the furnace to be used has a differential of plus or minus 10° F., or greater, a practice of aging for 6 hours at 350° F. is recommended. A somewhat lower elongation is obtained by the higher temperature-shorter time aging practices.

Unlike 24S-O, my product can be formed, hammered, rolled, or drawn, then solution and precipitation heat treated to develop maximum tensile properties in the "T" condition.

Tests have shown that sheets of my product have superior drawing characteristics to annealed 24S. Average Erichsen values obtained on R-301-O sheet are as follows:

|    | Gauge | No. of Tests | Erichsen |
|----|-------|--------------|----------|
| 40 | .040" | 12           | 8.54     |
|    | .051" | 12           | 8.72     |
|    | .064" | 18           | 9.06     |

The formability of sheets of my product is superior to that of 24ST or Pureclad 24S-T, offering an advantage in that a portion of those parts now requiring 24S-O or Pureclad 24S-O can be made using my product in the solution heat treated (W) condition, thereby eliminating subsequent heat treatment and distortion. For example, .064" R-301-W sheet can be bent 90° on a power brake both with and across grain over a radius of  $\frac{1}{8}$ " or 1T. Average Erichsen values obtained on R-301-W sheet are:

|    | Gauge | No. of Tests | Erichsen |
|----|-------|--------------|----------|
| 55 | .040" | 18           | 6.50     |
|    | .051" | 30           | 6.81     |
|    | .064" | 18           | 6.85     |
| 60 | .091" | 9            | 5.82     |

Spot welds made on my sheets have shown that the cladding alloy does not protrude into the elliptical fused zone; and have also shown excellent uniformity, along with good corrosion resistance both stressed and unstressed.

The Rockwell "E" hardness for the various tempers of my clad sheet have been determined as follows:

|    |         |            |
|----|---------|------------|
| 70 | R-301-O | 45 to 50   |
|    | R-301-W | 95 to 100  |
|    | R-301-T | 100 to 105 |

It is to be pointed out that R-301-T sheet possesses a harder surface than pure aluminum clad

sheet and subsequently is more resistant to scratching and abrading.

As stated above, in my product there is less difference in electrical potential between the core and the cladding as compared to the same alloy core and a pure metal cladding. Comparative potential measurements of my solution and precipitation heat treated sheet shows the following:

| Volts           | 10  |
|-----------------|-----|
| .064" core      | .72 |
| .064" cladding  | .82 |
| .064" composite | .82 |

The precipitation heat treatment of the tested sheet consisted of eighteen hours total time in Lindberg furnace at 320° F. preceded by solution heat treatment of twenty-two minutes in Lindberg furnace at 940° F. soaking nineteen minutes at 940° F. followed by cold water quench.

The potential measurements employed a saturated calomel electrode and solution, containing 57 grams sodium chloride and 100 cubic centimeters of 3% hydrogen peroxide solution per liter.

Even after severe corrosion tests my product retains substantially greater tensile properties than possessed by the said 24-S pure aluminum clad alloy. The following table shows examples, the treated sheets being of various gauges, the composition of the cladding being Si .70%, Mn .50%, Mg 1.00%, balance aluminum, and the cladding being 5% each side.

6 same gauge (.032") and under the same conditions, as follows:

|         | Per Cent Loss in Tensile Strength | Per Cent Loss in Yield Strength | Per Cent Loss in Elongation | Per Cent Loss in Weight |
|---------|-----------------------------------|---------------------------------|-----------------------------|-------------------------|
| 24S-T   | 5.99                              | 6.02                            | 70.3                        | 1.68                    |
| PC24S-T | .18                               | .26                             | 1.0                         | .32                     |

The corrosion tests applied to my sheets and 24S-T and P. C. 24S-T were calculated as equivalent to 2-4 years exposure to ocean salt spray mist (Hampton Roads).

Precipitation heat treatment, i. e. artificial aging, increases the strength of the core as well as cladding, and the corrosion resistance of the cladding is not materially lessened. Thus in .040" gauge maximum tensile strength was obtained, after solution heat treatment 15 minutes at 940 degrees F. with precipitation heat treatment about 20 hours at 320° F., or 12-14 hours at 340° F., or about 7 hours at 360° F.

Having described my invention, what I claim and desire to secure by Letters Patent is as follows:

1. A clad aluminum alloy composed of a core of a Duralumin type alloy having a cladding of an alloy composed substantially entirely of Si .50-.90%, Mn .25-.75%, Mg .80-1.2% and the balance aluminum, the alloys of the core and cladding having similar responsiveness to the same heat

TABLE I  
Corrosion tests on R-301-W and R-301-T sheet

| Guage | Temper | Tensile Strength, Lbs./Sq. Inch |          | Percent Change | Yield Strength, Lbs./Sq. Inch |          | Percent Change | Elongation, Percent in 2 Ins. |          | Percent Change | Loss in Weight, Percent |
|-------|--------|---------------------------------|----------|----------------|-------------------------------|----------|----------------|-------------------------------|----------|----------------|-------------------------|
|       |        | Original                        | Corroded |                | Original                      | Corroded |                | Original                      | Corroded |                |                         |
| .040" | R301-W | 61,900                          | 61,000   | -1.3           | 41,600                        | 40,900   | -2.7           | 19.3                          | 19.5     | +1.0           | -.92                    |
| .051" | R301-W | 60,200                          | 59,800   | -0.7           | 39,200                        | 38,300   | -2.3           | 20.3                          | 20.3     | 0              | -.56                    |
| .064" | R301-W | 60,700                          | 59,700   | -1.6           | 40,100                        | 39,800   | -0.7           | 19.2                          | 19.8     | +3.1           | -.18                    |
| .040" | R301-T | 66,900                          | 65,600   | -1.6           | 59,500                        | 58,200   | -2.2           | 9.0                           | 9.0      | 0              | -.75                    |
| .051" | R301-T | 68,000                          | 67,100   | -1.3           | 60,300                        | 60,600   | +0.5           | 9.5                           | 8.7      | -8.4           | -.46                    |
| .064" | R301-T | 66,900                          | 66,200   | -1.0           | 60,800                        | 59,400   | -0.7           | 10.0                          | 9.8      | -2.0           | -.24                    |

## NOTES

1. Corrosion consisted of a 6-hour immersion in a solution of 57 grams of sodium chloride 10 ml. of 30% hydrogen peroxide Balance of liter—distilled water

Specimens were cleaned prior to corrosion by immersion for 1 min. at 95 degrees C. in—  
50 ml. of concentrated nitric acid (70%)  
50 ml. of hydrofluoric acid (48%)  
Balance of liter—distilled water

- After cleaning, specimens were rinsed in distilled water, immersed one minute in concentrated nitric acid, rinsed in distilled water and dried. After corrosion, specimens were cleaned by immersion in 70% nitric acid, rinsed in distilled water and dried by air and dessication.
2. All of above specimens exhibited pitting type of attack only upon microscopic examination.
  3. Corrosion carried out at constant temperature of 75 degrees F.
  4. .040" R301-W sheet was heat treated in plant air furnace receiving a 12-minute soak at 930 to 945 degrees F. .051" and .064" R301-W sheet was heat treated in plant air furnace receiving a 15-minute soak at 930 to 945 degrees F. R301-W sheet was aged in plant air furnace, receiving an 18-hour soak at 320 degrees F.

The same corrosion tests applied to my clad sheets (R301-T) of .032" (5% each side) showed 65 the following maximum losses:

|        | Per Cent Loss in Tensile Strength | Per Cent Loss in Yield Strength | Per Cent Loss in Elongation | Per Cent Loss in Weight |
|--------|-----------------------------------|---------------------------------|-----------------------------|-------------------------|
| R301-T | 1.05                              | 2.15                            | 11.42                       | .39                     |

The above is comparative with corrosion resistance of 24S-T and Pureclad 24S-T sheets of the 75

treatments, there being not over .6% Fe in any impurity content present in the cladding alloy.

2. A clad aluminum alloy composed of a core of an alloy composed substantially entirely of Si .75-1.25%, Cu 4.0-5.0%, Mg .25-.55%, Mn .7-1.0% and the balance aluminum, the said core alloy having a cladding of an alloy composed substantially entirely of Si .50-.90%, Mg .8-1.2%, Mn .25-.75% and the balance aluminum, the alloys of the core and cladding having similar responsiveness to the same heat treatments, there being not over .75% Fe in any impurity content present

in the core alloy and not over .6% Fe in any impurity content present in the cladding alloy.  
THOMAS L. FRITZLEN.

| Number    | Name     | Date          |
|-----------|----------|---------------|
| 2,106,259 | Stockmar | Jan. 25, 1938 |
| 2,122,535 | Nock     | July 5, 1938  |

## REFERENCES CITED

The following references are of record in the file of this patent:

## UNITED STATES PATENTS

| Number    | Name  | Date          |
|-----------|-------|---------------|
| 1,805,448 | Frary | May 12, 1931  |
| 1,865,089 | Dix   | June 28, 1932 |

| Number  | Country | Date          |
|---------|---------|---------------|
| 207,559 | Sweden  | Feb. 16, 1940 |

| FOREIGN PATENTS                                                                                                            |  |  |
|----------------------------------------------------------------------------------------------------------------------------|--|--|
| Metals Handbook, 1939 Edition, Published by American Society For Metals, 7016 Euclid Avenue, Cleveland, Ohio, pp. 1270-71. |  |  |

## OTHER REFERENCES